# EUROPEAN PATENT APPLICATION

(11) **EP 1 447 146 A1**
(43) Date of publication of application: **18.08.2004**
(21) Application number: 04075418.6
(22) Date of filing: 10.02.2004
(51) Int. Cl.: B05D 7/02, B05D 7/00, B05D 5/06

(54) **Method for coating a surface, especially a plastic profile and coated plastic profile**

(30) Priority: 12.02.2003 BE 200300096
(71) Applicant: Deceuninck NV, 8830 Hooglede-Gits (BE)
(72) Inventor: Grymonprez, Wim, 8800 Roeselare (BE)
(74) Representative: Ostyn, Frans, Ing.

(57) **Abstract**

This invention relates to a method for lacquering a surface, a first layer of a product containing a coloured pigment and a second layer of a product containing a coloured pigment being successively applied to a surface, one covering the other, the second layer not containing no carbon black and the colour of the first layer and of the second layer together producing a predetermined colour. This predetermined colour being a colour belonging to the RAL-standard.

## Description

This invention relates to a method for lacquering a surface, a first layer of a product containing a coloured pigment and a second layer of a product containing a coloured pigment being successively applied to a surface, one covering the other, on the one hand, and to a section made of synthetic material made according to such a method, on the other hand.

The field of application of the invention is more particularly the surfaces of doors, windows or porches. The underlying material may be both thermosetting and thermoplastic synthetic material. For manufacturing the section made of synthetic material, in most cases use is made of polyvinyl chloride (PVC).

Sections made of a polymer matrix, such as PVC, for instance, are used more and more. They are used, for instance, for manufacturing window sections, doors, etc... The great advantage of such sections is their low weight and their resistance to corrosion.

On today's market there is a growing demand for coloured sections. These coloured sections are obtained by applying known techniques, such as, for instance, applying a coating by means of co-extrusion, etc...

However, practice has shown that under the influence of sunlight, more particularly of infrared radiation (IR) a heating-up occurs of the surface of sections made of synthetic material. It has been found that dark coloured (brown, green) sections, will heat up under the influence of infrared radiation till they almost reach their Vicat temperature. It has been found that window frame sections made of PVC (Vicat temperature 82°C), in countries were the sun is shining abundantly, for instance, in France and Spain, will heat up to a temperature lying between 70°C and 80°C.

Once sections made of synthetic material have reached their Vicat temperature, the polymer chains start to be redirected. Now as it is, when such sections are cooling down again, they will start to shrink, thus causing deformations.

In order to compensate this shrinkage, several solutions are used, for instance, metal reinforcing elements being inserted into the section. This has the disadvantage that the sections become much heavier.

Sometimes, reinforcing fibres are added to the polymer matrix, however they do have the disadvantage that the resistance to shock of the sections equipped with such reinforcing elements is strongly reduced, moreover these fibres are very expensive.

Recently new coatings have been developed however, such coatings being provided with "infrared reflecting pigments", because of which they will absorb less infrared radiation. These coatings do have the disadvantage that they have a low covering power on the one hand and will produce a difference in colour with respect to the RAL-standard on the other hand. The RAL-standard is an internationally agreed standard that is used to indicate identical colours, RAL 6009, for instance, stands for pine foliage and RAL 5012 for steel blue.

The purpose of the present invention is to provide a method for lacquering surfaces of synthetic material according to which less infrared radiation is absorbed by the polymer matrix, so that less deformation will occur and there will no longer be any difference in colour with respect to the RAL-standard.

The purpose of the invention is attained by providing a method for lacquering a surface, a first layer of a product containing a coloured pigment and a second layer of a product containing a coloured pigment being successively applied to the surface, one covering the other, the second layer containing no carbon black and the first and the second layer together producing a predetermined colour. Because of this a surface with a predetermined colour is obtained, absorbing far less infrared radiation.

In a preferred method of the invention the predetermined colour is a RAL-colour, because of which surfaces may be produced having the exact colour according to the RAL-standard. The great advantage of this method is that the method described in the present invention is universally applicable. Preferably, the colour of the first and the second layer both belong to the same RAL-group of colours.

In a particularly preferred method according to the invention, the second layer is applied before the first layer will be dry.

In a more particularly preferred method according to the invention, the first layer and/or the second layer are dispersed with polyamide particles, because of which a granular aspect is obtained.

In another preferred method according to the invention the said surface is a section made of synthetic material, preferably made of polyvinyl chloride.

Another object of the present invention is a section made of synthetic material, provided with at least two layers of coating with a coloured pigment, the upper layer containing no carbon black and in combination with the underlying layer producing a predetermined colour, this predetermined colour belonging to the RAL-standard. In a preferred embodiment, the colours of the two layers belong to the same RAL-colour group.

According to a preferred embodiment of the section made of synthetic material according to the invention, the underlying layer is a dark coating that under influence of the sun causes a rise in temperature of the surface with respect to the ambient temperature of minimum 65°C.

As it is, for instance, sections made of synthetic material of the colour RAL 6010 (grass green) may be produced, the chance that such coloured sections reach their Vicat temperature being much smaller.

According to a more particularly preferred embodiment of the section made of synthetic material according to the invention, the underlying layer is a semidark coating, that under the influence of the sun produces a rise in temperature of the surface ranging from 30°C to 50°C with respect to the ambient temperature.

For instance, sections made of synthetic material of the colour RAL 5007 (light blue) or, for instance, RAL 1013 (pearl white) may be produced, having far less chance to reach their Vicat temperature.

According to a most particularly preferred embodiment of the section made of synthetic material according to the invention, said sections are provided for manufacturing doors, windows and porches.

In order to further clarify the characteristics of the present invention and to indicate its additional advantages and particulars, a more detailed description of the method applied and of the section made of synthetic material produced according to this method will now follow. It will be obvious that nothing in the following description may be interpreted as a restriction of the protection of this invention demanded for in the claims.

In order to obtain coloured sections that will absorb the infrared radiation to a lesser extent, the section made of synthetic material has to be provided with a covering layer containing a coloured pigment (including carbon black) of liquid paint on a basis of thermoplastic resins, which paint contains a thermosetting polymer with hydroxyl and/or carboxyl groups, a hardener for interlacing the polymer and possibly containing a thermoplastic polyamide resin powder dispersed in the paint.

The product ensuring interlacing, also known as hardener, consists of aliphatic isocyanates. As an alternative it might also be aliphatic or cycloaliphatic, the use of diisocyanates and tri-isocyanates being preferred. In this case the combined polymer has a hydroxide and/or carboxyl/isocyanate function known as polyurethane.

Examples of polyamides are polyamide PA-6.6., polyamide-6.10. and polyamide PA-6.12. Mixtures are possible. usually they are PA-11, PA-12, PA-6/12 and/or PA-12.12., separated or as mixtures, in short, preferably polyamides having 10 to 13 carbon atoms per carbon amide group.

The powders are obtained by grinding or direct polymerization in order to obtain the desirable granulometric dimensions.
The final aspect of the first layer may be either a smooth structure or a granulated structure and any structure in between.

Preferably, the first layer is applied by means of a spray unit, the sections made of synthetic material being introduced into an automated spray unit, with an automatic conveying system. As a consequence of the continuous spraying, the visual aspect of the coloured surfaces is more uniform than when using a manual treatment.

Applying the first layer may be carried out in a number of successive steps, for instance, a first layer containing pigment (including carbon black) may be applied in two phases.

After the first layer having been applied, the second layer containing coloured pigment (the cold pigment layer) that contains no carbon black is applied wet-on-wet, i.e. without the first layer being dried. In actual practice it is usually the case that in most of the applications the grains of polyamide are dispersed in the top layer.

When both layers have been applied to the section made of synthetic material, they have to undergo a post hardening. This process sometimes is described as "curing". Preferably, this post hardening occurs within half an hour after the spraying operation and at a temperature of 80°C maximum. This is done, because it has been found that by not waiting too long after applying the coloured layers, the best results are obtained from an aesthetic point of view.

At temperatures over 80°C the chance that the elements made of synthetic material will be deformed becomes too great. In order to reduce the chance of a deformation to a minimum and yet to obtain a high quality, the temperature for this post hardening is preferably chosen between 40°C and 80°C.

After the two layers have been subjected to a curing process, a section made of synthetic material is obtained having the RAL-colour desired.

## Claims

1. Method for lacquering a surface, a first layer of a product containing a coloured pigment and a second layer of a product containing a coloured pigment being successively applied to a surface, one covering the other, **characterized in that** the second layer does not contain carbon black and **in that** the colour of the first and the second layer together will produce a predetermined colour.

2. Method for lacquering a surface according to claim 1, **characterized in that** said predetermined colour is a RAL-colour.

3. Method for lacquering a surface according to claim 1 or 2, **characterized in that** the colour of the first and of the second layer both belong to the same group of RAL-colours.

4. Method for lacquering a surface according to any one of the preceding claims, **characterized in that** the second layer is applied before the first layer has dried.

5. Method for lacquering a surface according to any one of the preceding claims, **characterized in that** the first layer and/or the second layer have been dispersed with polyamide particles.

6. Method for lacquering a surface according to any one of the preceding claims, **characterized in that** the said surface is a section made of synthetic material.

7. Method for lacquering a surface according to claim 6, **characterized in that** the said section made of synthetic material is preferably made of polyvinyl chloride.

8. Section made of synthetic material, provided with at least two layers of coating containing a coloured pigment, **characterized in that** the upper layer contains no carbon black and in combination with the underlying layer produces a predetermined colour.

9. Section made of synthetic material according to claim 8, **characterized in that** the predetermined colour of the said section made of synthetic material belongs to the RAL-standard.

10. Section made of synthetic material according to claim 8 or 9, **characterized in that** the said layers both belong to the same group of RAL-colours.

11. Section made of synthetic material according to any one of the claims 8 up to and including 10, **characterized in that** the underlying layer is a dark coating that itself, under the influence of the sun, causes a rise in temperature of the surface of at least 65°C.

12. Section made of synthetic material according to any one of the claims 8 up to and including 10, **characterized in that** the underlying layer is a semidark coating that under the influence of the sun, causes a rise in temperature of the surface lying between 30°C and 50°C.

13. Section made of synthetic material according to any one of the claims 8 up to and including 12, **characterized in that** the sections made of synthetic material are doors, windows or porches.
